

R. P. PERRY.  
HYDROCARBON COKE.  
APPLICATION FILED SEPT. 1, 1915.

1,257,959.

Patented Feb. 26, 1918.



Ray Potter Perry Inventor

By his Attorneys

Messrs. Leverett

# UNITED STATES PATENT OFFICE.

RAY POTTER PERRY, OF MONTCLAIR, NEW JERSEY, ASSIGNOR TO THE BARRETT COMPANY, OF NEW YORK, N. Y., A CORPORATION OF WEST VIRGINIA.

## HYDROCARBON COKE.

1,257,959.

Specification of Letters Patent. Patented Feb. 26, 1918.

Original application filed May 19, 1915, Serial No. 29,219. Divided and this application filed September 1, 1915. Serial No. 48,384.

*To all whom it may concern:*

Be it known that RAY POTTER PERRY, a citizen of the United States, and resident of Montclair, county of Essex, and State of New Jersey, has invented a certain new and useful Hydrocarbon Coke, of which the following is a specification, this application being for an article of manufacture and constituting a divisional application of his pending application, Serial No. 29,219, filed May 19, 1915, and patented March 14, 1916, No. 1,175,079.

The object of my invention is to produce a new and useful product from coal tar, coal tar pitch, petroleum, asphalt, and similar hydrocarbons, which either are liquid in their normal condition or can be liquefied by heat to render them adaptable to my new process of converting them into coke, by driving off by means of heat all or practically all of their volatile constituents.

Known methods of coking solids such as coal, wood, etc., in general consist in placing the material to be treated in a chamber, such as a gas retort, beehive coke oven or by-product coke oven, and heating this material externally, or often internally, by combustion of a portion of the material, to such temperature and for such period as is required to drive off all or practically all of its volatile matter, leaving a coke residue. The use of such retorts or chambers has been attempted for the coking of such materials as coal tar pitch, but it presents certain disadvantages in addition to the evident ones incidental to any intermittent operation. An additional disadvantage for the coking of such a material as coal tar pitch, in an oven of this type is that at a certain stage in the process decomposition takes place with the rather sudden formation of a considerable volume of gas, which causes the material to foam and tend to overflow from the chamber, or oven, through the vapor pipe. The increase of volume incident to the decomposition is so great that it is necessary to use a much smaller quantity of pitch in an oven of a given size than is customary in coking coal, and this results in requiring larger investment for a given output.

In the petroleum industry it has been usual to distil the petroleum oil in cylindrical steel stills, usually horizontal, to drive off the naphtha, gasolene, illuminating and

lubricating oils, etc., leaving as a residue in 55 the still a petroleum tar or pitch. If desired the heating of the still is continued until practically all of the volatile matter has been driven off, leaving a coke residue on the bottom of the still, or the petroleum tar or 60 pitch in a hot, liquid condition is transferred to other smaller stills where the heating is continued until the desired coke is obtained. It has been found that the high heat necessary for coking in this manner burns out the 65 still bottoms in a relatively short time, requiring frequent and expensive repairs. This burning of the steel forming the still bottom is hastened by the fact that the coke formed immediately adjoining the bottom 70 on the inside surface acts as a heat insulator and requires the application of more intense heat in order to transmit sufficient heat to coke satisfactorily the tar or pitch not in contact with the still bottom. This burning 75 action of the steel is somewhat similar to the burning of boiler plates when covered by a layer of scale. After the coke has been formed it is necessary to allow the still and setting to cool sufficiently so that the still 80 can be opened and workmen enter with picks and shovels to loosen and remove the coke. This obviously results in a great waste of time as well as loss of heat.

To overcome the disadvantages necessarily 85 incident to any of the processes heretofore employed, I have invented a continuous process by means of which I accomplish coking by heating the material in liquid form in comparatively thin films on a moving 90 surface as hereinafter described and claimed.

One preferred form of apparatus for carrying out my invention is shown diagrammatically in the drawing forming part of this specification, in which A is a chamber 95 in which is mounted a hollow cylinder 2 revolving on a shaft 3 in the direction shown by the arrow. The material to be treated is delivered through the pipe 4 from a source of supply (not shown) into the pan 5 into 100 which the cylinder 2 dips. As the cylinder revolves a thin film of the liquid 6 is carried along on the outer surface of said cylinder. The interior surface of the cylinder 2 is heated by any convenient means, as for example, gas jets 7. The chamber A is provided with a vapor pipe 8 which leads to a vapor condensing system (not shown). The

scraper 9 is set in contact with the outer surface of the cylinder 2 and serves to remove the film of coke 10 which has been formed thereon depositing it in a pile 11 upon the 5 valve 12 which may be opened when desired to allow the accumulated coke to drop into the storage chamber from which it is from time to time removed by opening the bottom 14.

- 10 The operation is as follows: The cylinder is heated internally to the desired temperature, and is revolved slowly in the direction indicated by the arrow. The surface D of the cylinder 2 dips into the liquid 6 in the 15 pan 5 and continuously picks up a thin film of the liquid. The heat transmitted by the surface of the cylinder 2 causes the volatile matter, or a large part of the same, to be evaporated from the liquid, the vapors escaping through the vapor pipe 8 to the condensing system, (not shown). If desired 20 vacuum may be applied to the condensing system to facilitate removal of the vapors, and to lower the temperature required for 25 evaporating the volatile matter from the liquid. The two valves 12 and 13 are provided in order not to break the vacuum which may be employed in the process, each valve serving to prevent the admission of 30 air to the cylinder when the other valve is opened to dump its contents.

As the liquid cokes, decomposition takes place, causing the film of liquid to foam, as indicated by the increased thickness of the 35 film at the top of the cylinder. By the time it reaches the scraper 9 the desired amount of volatile matter has been driven off by heat and the scraper removes the film of coke which falls and accumulates on the 40 valve 12. From time to time this valve is opened and all the accumulated coke falls to the lower valve 13 and from time to time is removed by opening this valve.

I may reverse the process and apply the 45 heat to the outside of the cylinder and the liquid to be coked to the interior surface of the cylinder but this is a less convenient method and is not recommended in practice. Also instead of picking up a film by causing 50 the surface of the cylinder to dip in a pan

containing the liquid to be coked I may employ any other convenient means, as for example by causing the liquid to flow on to the surface of the cylinder from above or by spraying it on such surface, or any other 55 convenient method may be employed to supply a thin film of the liquid to be coked to the cylinder or other moving surface.

The degree of heat necessary to reduce liquefied tar so as to gasify at least 85% of 0 the volatile material and reduce the residuum to a coke, is in excess of 1000° F. under atmospheric pressure, which can of course be reduced materially by treatment under 65 vacuum. As the liquid film which adheres to the surface of the drum is very thin, the layer or sheet of coke when removed is also thin and fragile, crumbling into small irregular fragments which are in condition 70 for molding into electrodes or to be utilized in other manufacturing operations, or if more finely divided material is desired the crushing or grinding operation is a very easy and simple operation, as compared with the pulverizing of ordinary coke fused into 75 large masses.

Having thus described my invention, what I claim and desire to secure by Letters Patent is:—

1. The herein described product consisting essentially of irregular scales of coke. 80
2. The herein described product consisting substantially entirely of irregular scales of coke. 85
3. The herein described homogeneous product consisting essentially of irregular scales of coke. 90
4. The herein described product consisting essentially of irregular porous scales of coke. 95
5. The herein described product consisting essentially of irregular scales of coke containing very little volatile matter.
6. The herein described product consisting essentially of irregular scales of coke containing less than 15% of volatile matter. 95

Signed at New York, in the county of New York and State of New York, this 28 day of August, 1915.

RAY POTTER PERRY.